# EUROPEAN PATENT SPECIFICATION

(11) **EP 3 652 363 B1**
(45) Date of publication and mention of the grant of the patent: **23.06.2021**
(21) Application number: 18735324.8
(22) Date of filing: 05.07.2018
(51) Int. Cl.: C25D 11/22, C25D 11/24

(54) **AN ALUMINIUM ALLOY ROLLED PRODUCT WITH INTENSE IRIDISCENT COLORS**
WALZPRODUKT AUS ALUMINIUMLEGIERUNG MIT INTENSIV IRISIERENDEN FARBEN
PRODUIT LAMINÉ EN ALLIAGE D'ALUMINIUM À COULEURS IRIDESCENTES INTENSES

(30) Priority: 10.07.2017 FR 1756527
(43) Date of publication of application: 20.05.2020
(73) Proprietor: Constellium Rolled Products Singen GmbH & Co.KG, 78224 Singen (DE)
(72) Inventor: SAFRANY, Jean-Sylvestre, 38500 Voiron (FR); FAIHY, David, 38140 Apprieu (FR)
(74) Representative: Constellium - Propriété Industrielle
(86) International application number: PCT/EP2018/068242
(87) International publication number: WO 2019/011778

(56) References cited:
- WO-A1-2017/013607
- US-A1- 2008 311 362
- US-A1- 2015 259 818
- US-A1- 2016 362 808
- PASTORE G ET AL: "Electrocolouring of anodized aluminium with copper: Effect of porous and barrier oxide film thicknesses", THIN SOLID FILMS, ELSEVIER, AMSTERDAM, NL, vol. 173, no. 2, 15 June 1989 (1989-06-15) , pages 299-308, XP025848125, ISSN: 0040-6090, DOI: 10.1016/0040-6090(89)90146-6 [retrieved on 1989-06-15]
- I. DE GRAEVE ET AL: "Colour simulation and prediction of complex nano-structured metal oxide films", SURFACE AND COATINGS TECHNOLOGY, vol. 205, no. 19, 1 June 2011 (2011-06-01) , pages 4349-4354, XP055450899, AMSTERDAM, NL ISSN: 0257-8972, DOI: 10.1016/j.surfcoat.2011.03.018

## Description

### FIELD OF THE INVENTION

The present invention relates to decorative aluminium rolled products having iridescent colors.

### BACKGROUND OF THE INVENTION

Various aluminium alloys are used in the form of rolled products for decorative applications such as cosmetic packaging, automotive trims (exterior and interior), interior design, sound system and consumer electronics.

Obtain iridescent colors on aluminium rolled products is known. By iridescent colors it is meant that the color changes as a function of the incident angle. In particular, it may be obtained on anodized aluminium having porous anodic oxide films obtained in various electrolytes (sulfuric, phosphoric, oxalic acid etc.). As shown in Figure 1, porous anodic oxide films consist of two layers, a porous thick outer layer 22 and an inner layer which is dense and dielectrically compact called the barrier layer 21. The iridescent phenomenon is due to interference between the light reflected on the oxide surface and the light reflected on a metal/oxide interface. At different incident angles V, as illustrated in Figure 1, different wavelengths of light have either positive or negative interference resulting in different colors being perceived.

Iridiscent colors may be observed on porous anodic oxide films. In the article "Optical properties and color generation mechanism of porous anodic alumina films" Applied Surface Science 258 (2011) 1826-1830 examples are provided of iridescent anodic aluminum oxide films obtained on high purity aluminum foils by phosphoric acid anodizing. The phenomenon appears to be enhanced if the porous anodic oxide film is colored.

In the article "Synthesis and properties of iridescent Zn-containing anodic aluminum oxide films" - Thin Solid Films 586 (2015) 8- 12, examples are provided of iridescent anodic aluminum oxide films obtained on high purity aluminum foils by phosphoric acid anodizing followed by Zn deposition.

In the article "Synthesis of iridescent Ni-containing anodic aluminum oxide films by anodization in oxalic acid" - Optical Materials 52 (2016) 107 - 110, examples are provided of iridescent anodic aluminum oxide films obtained by acid anodizing followed by Ni electro deposition.

The patent application WO2017/013607 relates to a structural colouration method for colouring an aluminium substrate, exemplified by alloy 6061, which comprises forming a nano structure of one-dimensional photonic crystals by means of a process of periodic current pulse anodisation, the colour obtained depending on the application time of the maximum and/or minimum current density of the pulse, and the colour varying with the angle of observation.

In the article "Electrocolouring of anodized aluminium with copper:effect of porous and barrier oxide film thickness", G. Pastore et al Thin Solid Films, 173 (1989) 299-308, is described the effect of the thickness of both porous and compact films of aluminium, exemplified by alloy 6063, anodized in 15% H₂SO₄ on the electrocolouring process using copper sulphate and magnesium sulfate solutions.

In the article "Colour simulation and prediction of complex nano-structured metal oxide films Test case : Analysis and modeling of electro-coloured anodized aluminium", I. De Graeve et al. Surface and Coatings Technology 205 (2011) 4349-4354, is described an optical modeling procedure to predict and model the colour of electro-coloured anodized aluminum exemplified by an aluminum AA5005 having 0.7 wt.% Fe and 0.3 wt.% Si.

Patent application US2016/0362808 describes a formed aluminum article, exemplified by alloys 6061 and 6063, in which pores formed by anodic oxidation are filled with a pigment, the formed aluminum article having an adequately colored film.

The colors can be adjusted by modifying the anodizing and coloring parameters, but for typical anodizing quality, e.g. high purity foils such as those described in the mentioned articles or more generally on 1XXX series alloys, the overall coloring effect remains light.

There is thus a need to obtain decorative aluminium rolled products with strong iridescent colors.

### SUMMARY OF THE INVENTION

An object of the invention is an anodized decorative rolled product made of an aluminum alloy consisting of, in weight %,
Mg : 0 - 1.5,
Mn : 0 - 1.5,
With Mg + Mn : 0.5 - 3
and wherein either Mn : 0.8 - 1.5 or Mg : 0.5 - 1.1 and Mn ≤ 0.2,
Si : ≤ 0.6,
Fe : ≤ 0.8,
Ti : ≤ 0.1,
Cu : ≤ 0.3,
Cr : ≤ 0.1,
Zn : ≤ 0.25,
Zr : ≤ 0.1,
other elements ≤ 0.05 each and ≤ 0.15 in total, remainder aluminium,
wherein the rolled product has a porous anodic oxide film which is colored electrochemically or chemically and wherein the color of the decorative sheet is different if viewed at an incidence angle 0° and at an incidence angle of 45° and wherein the porous anodic oxide film is covered by a sol-gel coating preferably comprising silicon.

Another object of the invention is a method to make an anodized decorative rolled product according to the invention comprising the steps of
- casting an aluminum alloy according to the invention to form an ingot;
- reheating and/or homogenizing the ingot preferably at a temperature from 460°C to 560°C,
- hot rolling the ingot to a hot rolling final thickness preferably at a temperature from 350 to 500°C,
- cold rolling to obtain a cold rolled product, with a preferred final thickness from 0.2 to 2 mm and preferably from 0.5 to 0.8 mm,
- optionally annealing said cold rolled product preferably at a temperature from 200 to 300 °C,
- cleaning said cold rolled product, preferably with a solvent or an aqueous cleaner containing surfactants,
- optionally providing a matt or bright aspect for example by satin matt etching or by chemical/electrochemical brightening,
- anodizing said cold rolled product in sulfuric acid, phosphoric acid or oxalic acid or a combination thereof to obtain a porous anodic oxide film,
- coloring said porous anodic oxide film by electrochemical deposition preferably of at least one of Zn, Ni, Sn, Co, Cu, Ag of or chemical deposition preferably of at least one dye among an azo dye, an anthraquinone dye, an indigo dye,
- rinsing with deionized water,
- optionally sealing the porous anodic oxide film by hydrothermal sealing, cold sealing or a combination thereof,
- drying,
- coating the porous anodic oxide film by depositing a sol-gel precursor followed by evaporation and/or curing.

### DESCRIPTION OF THE FIGURES

Figure 1 : Interference between the light reflected on the oxide surface and the light reflected on a metal/oxide interface, for an anodic porous alumina on an aluminium surface.

### DESCRIPTION OF THE INVENTION

All aluminium alloys referred to in the following are designated using the rules and designations defined by the Aluminum Association in Registration Record Series that it publishes regularly, unless mentioned otherwise.

Unless otherwise indicated, all the indications relating to the chemical composition of the alloys are expressed as a mass percentage by weight based on the total weight of the alloy. In the formula Mg + Cu, Mg and Cu means the percentage by weight of Mg and Cu, respectively.

Metallurgical tempers referred to are designated using the European standard EN-515.

The inventors have found that by using alloys having a specific composition, and in particular including additions of Mg and/or Mn it is possible to obtain decorative aluminium rolled products with strong iridescent colors

According to the invention, an anodized decorative rolled product with strong iridescent colors can be obtained with rolled product made of an aluminum alloy consisting of, in weight %,
Mg : 0 - 1.5,
Mn : 0 - 1.5,
with Mg + Mn : 0.5 - 3
and wherein either Mn : 0.8 - 1.5 or Mg : 0.5 - 1.1 and Mn ≤ 0.2,
Si : ≤ 0.6,
Fe : ≤ 0.8,
Ti : ≤ 0.1,
Cu : ≤ 0.3,
Cr : ≤ 0.1,
Zn : ≤ 0.25,
Zr : ≤ 0.1,
other elements ≤ 0.05 each and ≤ 0.15 in total, remainder aluminium,
wherein the rolled product has a porous anodic oxide film which is colored electrochemically or chemically and wherein the color of the decorative sheet is different if viewed at an incidence angle 0° and at an incidence angle of 45° and wherein the porous anodic oxide film is covered by a sol-gel coating preferably comprising silicon.

The presence of Mn and/or Mg containing precipitates in the alloy surprisingly enhances the colors and iridescent properties.

Presence of Si further improves the strength of colors in some instances. Advantageously the Si content is at least 0.03 wt.%. Excessive Si content can however be detrimental to formability. Preferably the Si content is at most 0.3 wt.% and preferably at most 0.25 wt.% and more preferably at most 0.2 wt.%.

Similarly presence of Fe further improves the strength of colors in some instances. Advantageously the Fe content is at least 0.02 wt.%. Excessive Fe content can however be detrimental to formability. Preferably the Fe content is at most 0.5 wt.%, more preferably at most 0.4 wt.% and preferentially at most 0.2 wt.%. Preferably Fe is at most 0.5 wt.% and Si is at most 0.3 wt.%. The other elements which have a content of ≤ 0.05 wt.% each and ≤ 0.15 wt.% in total, are undesirable impurities.

In a first embodiment, the alloy contains from 0.8 to 1.5 wt.% Mn and is preferably an alloy from the 3XXX series. Preferred alloys in this first embodiment are AA3103, AA3104 and AA3005. Preferably in the first embodiment the Mg content is at most 1.3 wt.% and preferably at most 0.6 wt.%

In a second embodiment the Mn content is at most 0.2 wt.% and the Mg content is from 0.5 to 1.1 wt.%. In this second embodiment the alloy is preferably an alloy from the 5XXX series. This second embodiment is advantageously also combined with a Si content of at most 0.2 wt.%, preferably at most 0.1 wt.% and most preferably at most 0.04 wt.%. This second embodiment is advantageously also combined with a Fe content of at most 0.2 wt.%, preferably at most 0.1 wt.% and most preferably at most 0.06 wt.%.Preferred alloys in this second embodiment are AA5005, AA5505 and AA5657.

The method to make an anodized decorative rolled product according according to the invention comprises the steps of
- casting an aluminum alloy according to the invention to form an ingot;
- reheating and/or homogenizing the ingot preferably at a temperature from 460°C to 560°C,
- hot rolling the ingot to a hot rolling final thickness preferably at a temperature from 350 to 500°C,
- cold rolling to obtain a cold rolled product, with a preferred final thickness from 0.2 to 2 mm and preferably from 0.5 to 0.8 mm,
- optionally annealing said cold rolled product preferably at a temperature from 200 to 300 °C,
- cleaning said cold rolled product, preferably with a solvent or an aqueous cleaner containing surfactants,
- optionally providing a matt or bright aspect for example by satin matt etching or by chemical/electrochemical brightening,
- anodizing said cold rolled product in sulfuric acid, phosphoric acid or oxalic acid or a combination thereof to obtain a porous anodic oxide film,
- coloring said porous anodic oxide film by electrochemical deposition preferably of at least one of Zn, Ni, Sn, Co, Cu, Ag of or chemical deposition preferably of at least one dye among an azo dye, an anthraquinone dye, an indigo dye,
- rinsing with deionized water,
- optionally sealing said porous anodic oxide film by hydrothermal sealing, cold sealing or a combination thereof,
- drying,
- coating the porous anodic oxide film by depositing a sol-gel precursor followed by evaporation and/or curing.

Typical surfactants are anionic such as carboxylates or sulphonates, nonionic such as ethoxylated aliphatic alcohols, cationic such as quaternary ammonium salts or amphoteric such as aliphatic aminocarboxylic acid salts.

The porous outer layer obtained from acid anodizing can be schematically represented as a closed-packed array of hexagonally arranged cells containing pores in each cell-center. Figure 1 illustrates a cross section of a porous anodic oxide film 2 on aluminium an aluminium substrate 1, comprising a barrier layer 21 and a porous outer layer 22. The porous anodic oxide film is characterized by given parameters such as a pore diameter, interpore distance (cell diameter) of the porous outer layer and the barrier layer thickness. The porous anodic oxide film of the products according to the invention exhibit a barrier layer with a thickness advantageously from 15 to 25 nm, in order to obtain the desired iridiscent colors. The porous anodic oxide film total thickness is advantageously between 1 and 10 µm.

Typically, a sulfuric anodizing can be achieved at 1-1,5A/dm² at 20°C, providing an approximately 21 nm thick barrier layer, the anodizing time being adjusted to vary the coloring effect,

The coloring dyestuff concentration may vary from 0.1 to 10g/L, depending on the color and the required darkness. The temperature is usually in the range of 50 to 60°C, with some exceptions working at lower temperature.

According to the invention the porous anodic oxide film is coated by depositing a sol-gel precursor followed by evaporation and/or curing to obtain a sol-gel coating. The present inventors observed that surprisingly the sol-gel coating does not alter the iridescent appearance, probably because of its specific optical properties. The sol-gel coating protects the porous anodic film from scratches, fingerprints, and other surface deffects. On the contrary, conventional coatings such as clear lacquer does not allow not to keep the iridescent aspect.

Preferably the sol-gel precursor is made from a mixture of a polysiloxane, preferably prepared from an alcoholic solution of silane, more preferably from an alcoholic solution of an alkoxysilane, and an aqueous solution of colloidal silica. The sol-gel precursor is advantageously prepared from two solutions A and B, solution A being an alcoholic solution of one or more alkoxysilanes, the alcohol used as solvent being methanol, ethanol, propanol, preferably isopropanol, butanol or a combination thereof, the alkoxysilanes being described by the general formula XnSi(OR)4-n wherein "R" is a simple alkyl, preferably chosen in the group consisting of methyl, ethyl, propyl and butyl and "X" is also an alkyl, preferably selected from the group consisting of methyl, ethyl, propyl and butyl; solution B being a solution of colloidal silica dissolved in water. Advantageously the alkoxysilanes belong to the group comprising tetramethoxysilane (TMOS), tetraethoxysilane (TEOS) and methyl trimethoxysilane (MTMOS). Preferably solution A contains 25 - 35 wt% TEOS and 15 - 25 wt% MTMOS, both dissolved in 40 - 60 wt% isopropyl alcohol. Advantageously solution B is set with an acid, preferably with nitric acid (HNO3), to a pH value between 2.0 and 4, preferably between 2.5 and 3.0 and more preferably close to 2.7. Advantgeously the alkali content of the silica is less than 0.04 wt % Na₂O.

Preferably the deposition of the sol-gel precursor is carried out by immersion. Advantageoulsy the sol-gel coating thickness is comprised between 2 and 4 µm. Preferably, the sol-gel coating contains a small quantity of organic compounds, for example the carbon content of the coating as measured by XPS (X-Ray Photoelectron Spectrometry) is less than 10 atomic % as measured by concentration profile through the sol-gel coating. Preferably curing of the sol-gel is done at a temperature comprised between 150 and 250 °C during 30 to 60 seconds.

The product of the invention is particularly useful for decorative applications such as cosmetic packaging, automotive trims (exterior and interior), interior design, sound system and consumer electronics.

### EXAMPLE

### Example 1 (reference example)

In this example, rolled products made of several alloys have been tested for color anodizing.

The composition of the alloys is provided in Table 1

**Table 1, Typical composition of alloys in wt.%**

| alloy | Si | Fe | Cu | Mn | Mg | Cr | Zn | Ti | Zr | Mg+Mn |
|---|---|---|---|---|---|---|---|---|---|---|
| 1070 | 0,01 | 0,12 | 0,002 | 0,002 | 0,002 | 0,002 | 0,002 | 0,002 | 0,002 | 0,004 |
| 5657 | 0,04 | 0,06 | 0,04 | 0,002 | 0,7 | 0,002 | 0,002 | 0,002 | 0,002 | 0,702 |
| 5505 | 0,04 | 0,03 | 0,002 | 0,002 | 0,8 | 0,002 | 0,002 | 0,002 | 0,002 | 0,802 |
| 3103 | 0,20 | 0,5 | 0,002 | 1,1 | 0,002 | 0,002 | 0,002 | 0,002 | 0,002 | 1,102 |
| 3104 | 0,21 | 0,35 | 0,2 | 0,9 | 1,3 | 0,008 | 0,002 | 0,01 | 0,002 | 2,2 |

The products received a surface treatment as follows :
- Solvent cleaning with Methyl-Ethyl Ketone on flat samples
- Deionized water rinse
- Anodizing with sulphuric acid 180g/L, at 20°C, for 1 to 2 min under a DC current of 1 A/dm²
- Deionized water rinse
- Electrolytic coloring : with nickel sulphate 30g/L, boric acid 30g/L, ammonium sulphate 15g/L, 35°C, 2 min 19V AC current or chemical coloring with an azo dye chromium complex : Sanodal® Black 2LW (1g/L), with an azo dye copper complex : Sanodure® Fast Gold L (3g/L), and with an anthraquinone dye :Sanodye® Blue 2LW (3g/L) at 60°C during 2 min,
- Deionized water rinse
- drying

The resulting samples were observed at different incident angles. The intensity of colors was classified through comparison with reference samples and scaled from 1 : light to 3 : strong.

The results are provided in Table 2

**Table 2 - Results obtained**

| Alloy | Anodizing duration (min) | coloring | Color (intensity) at incident angle | | |
|---|---|---|---|---|---|
| | | | 0° | 45° | 90° |
| 1070 | 1 | electroly tic | Green (1) | Pink(1) | Green-Blue (1) |
| 1070 | 2 | Chemical (black) | Pink (1) | Blue-Green (1) | uncolore d |
| 5657 | 2 | Chemical (black) | Pink (2) | Blue-Green (2) | uncolore d |
| 5505 | 2 | Chemical (gold) | Gold-green (2) | Gold-pink (2) | Gold (2) |
| 3103 | 2 | Chemical (blue) | Blue (2) | Pink (2) | Blue (2) |
| 3103 | 1,5 | Chemical (blue) | Pink (2) | Blue (2) | Pink (2) |
| 3104 | 1 | electroly tic | Green (3) | pink (3) | Green-Blue (3) |
| 3104 | 2 | Chemical (black) | Pink (3) | Blue-green (3) | Pink (2) |

| | | | | | |
|---|---|---|---|---|---|
| Intensity : 1 : light, 2 : medium, 3 : strong | | | | | |

Coloring with alloys according to the invention enables obtention of strong iridescent colors, ranging from 2 to 3.

### Example 2

The sample of example 1 made of alloy 5657 is protected by a sol-gel coating.

The sol-gel solution applied by immersion consists of the mixture of a solution A and a solution B.

Anhydrous solution A comprises a mixture of unhydrolyzed siloxanes and alcohols:
50% by weight of isopropanol
30% by weight of tetraethylorthosilicate (TEOS)
20% by weight of trimethoxymethylsilane (MTMOS)
The aqueous solution B comprises: 25% by weight of colloidal silica and 75% by weight of water.

The pH of solution B is modified to reach 2.5 by addition of acid such as, for example, HNO3. The silica must have the lowest possible alkaline content, preferably less than 0.04 mass% of Na2O.

Solution A is mixed with solution B in the presence of nitric acid with continuous stirring and leads to a hydrolysis and condensation reaction bringing the mixture to a gel state. Solutions A and B are mixed with a weight ratio of preferably 7: 3. The mixture is preferably maintained at a pH value of between 2 and 4, preferably 2.5 to 3.0, and most preferably 2.7. The pH value is corrected by addition of acid, preferably nitric acid.

After mixing solutions A and B for 6 hours, the resulting solution is filtered. The filtration may, for example, be carried out using polypropylene filters with a mesh size of 1 micron. Before use, the solution is left standing for 12 to 22 hours before being applied to the substrate to form the protective deposit.

The baking of the deposit is carried out at a temperature of 150 to 250 ° C for 30s to 60s. The thickness of the deposit is preferably 2 to 4 µm and contains only very few organic compounds (less than 10 at%, measured by depth profile in XPS).

The strong iridescent coloring of the alloy according to the invention is not modified by the sol-gel coating, which is suprising because irridescence is based on interference phenomena and the addition of a thin coating is expected to affect coloring. Moreover the surface is well protected mechanically by the sol-gel coating.

## Claims

1. An anodized decorative rolled product made of an aluminum alloy consisting of, in weight %,
Mg : 0 - 1.5,
Mn : 0 - 1.5,
with Mg + Mn : 0.5 - 3, and wherein
either Mn : 0.8 - 1.5
or Mg : 0.5 - 1.1 and Mn ≤ 0.2,
Si : ≤ 0.6,
Fe : ≤ 0.8,
Ti : ≤ 0.1,
Cu : ≤ 0.3,
Cr : ≤ 0.1,
Zn : ≤ 0.25,
Zr : ≤ 0.1,
other elements ≤ 0.05 each and ≤ 0.15 in total, remainder aluminium,
wherein the rolled product has a porous anodic oxide film which is colored electrochemically or chemically and wherein the color of the decorative sheet is different if viewed at an incidence angle 0° and at an incidence angle of 45° and **characterized in that** the porous anodic oxide film is covered by a sol-gel coating preferably comprising silicon.

2. A product according to claim 1 wherein
Fe is at most 0.5 wt.% and Si is at most 0.3 wt.%.

3. A product according to claim 1 or claim 2 wherein
Mn is at most 0.2 wt, Si is at most 0.1 wt.% and Fe is at most 0.2 wt.%.

4. A product according to claim 1 or claim 2 wherein
Mn : 0.8 - 1.5 wt.% and wherein the Mg content is at most 1.3 wt.% and preferably at most 0.6 wt.%.

5. A product according to anyone of claims 1 to 4 wherein the Si content is at least 0.03 wt.%.

6. A product according to anyone of claims 1 to 5 wherein the Fe content is at least 0.02 wt.%.

7. A product according to any of claims 1 to 6 wherein the barrier layer of the porous anodic oxide film has a thickness from 15 to 25 nm.

8. A product according to any of claims 1 to 7 wherein the porous anodic oxide film comprises at least one of Zn, Ni, Sn, Co, Cu, Ag.

9. A product according to any of claims 1 to 7 wherein the porous anodic oxide film comprises at least one dye among a azo dye, an anthraquinone dye, an indigo dye.

10. A method to make an anodized decorative rolled product according to anyone of claims 1 to 9 comprising the steps of
- casting an aluminum alloy according to anyone of claims 1 to 6 to form an ingot;
- reheating and/or homogenizing the ingot preferably at a temperature from 460°C to 560°C,
- hot rolling the ingot to a hot rolling final thickness preferably at a temperature from 350 to 500°C,
- cold rolling to obtain a cold rolled product, with a preferred final thickness from 0.2 to 2 mm and preferably from 0.5 to 0.8 mm,
- optionally annealing said cold rolled product preferably at a temperature from 200 to 300 °C,
- cleaning said cold rolled product, preferably with a solvent or an aqueous cleaner containing surfactants,
- optionally providing a matt or bright aspect for example by satin matt etching or by chemical/electrochemical brightening,
- anodizing said cold rolled product in sulfuric acid, phosphoric acid or oxalic acid or a combination thereof to obtain a porous anodic oxide film,
- coloring said porous anodic oxide film by electrochemical deposition preferably of at least one of Zn, Ni, Sn, Co, Cu, Ag of or chemical deposition preferably of at least one dye among an azo dye, an anthraquinone dye, an indigo dye,
- rinsing with deionized water,
- optionally sealing the porous anodic oxide film by hydrothermal sealing, cold sealing or a combination thereof,
- drying,
- coating the porous anodic oxide film by depositing a sol-gel precursor followed by evaporation and/or curing.

11. A method according to claim 10 wherein the sol-gel precursor is made from a mixture of a polysiloxane, preferably prepared from an alcoholic solution of silane, more preferably from an alcoholic solution of an alkoxysilane, and an aqueous solution of colloidal silica.

12. A method according to claim 11 wherein the sol-gel precursor is prepared from two solutions A and B, solution A being an alcoholic solution of one or more alkoxysilanes, the alcohol used as solvent being methanol, ethanol, propanol, preferably isopropanol, butanol or a combination thereof, the alkoxysilanes being described by the general formula XnSi(OR)4-n wherein "R" is a simple alkyl, preferably chosen in the group consisting of methyl, ethyl, propyl and butyl and "X" is also an alkyl, preferably selected from the group consisting of methyl, ethyl, propyl and butyl;
solution B being a solution of colloidal silica dissolved in water.

13. A method according to claim 12 wherein said alkoxysilanes belong to the group comprising tetramethoxysilane (TMOS), tetraethoxysilane (TEOS) and methyl trimethoxysilane (MTMOS).

14. A method according to claim 13, wherein the solution A contains 25 - 35 wt% TEOS and 15 - 25 wt% MTMOS, both dissolved in 40 - 60 wt% isopropyl alcohol.

## Patentansprüche

1. Eloxiertes dekoratives Walzprodukt aus einer Aluminiumlegierung, bestehend aus, in Gew.-%,
Mg: 0 - 1,5,
Mn: 0 - 1,5,
mit Mg + Mn: 0,5 - 3, und wobei
entweder Mn: 0,8 - 1,5
oder Mg: 0,5 - 1,1 und Mn ≤ 0,2,
Si: ≤ 0,6,
Fe: ≤ 0,8,
Ti: ≤ 0,1,
Cu: ≤ 0,3,
Cr: ≤ 0,1,
Zn: ≤ 0,25,
Zr: ≤ 0,1,
weitere Elemente jeweils ≤ 0,05 und ≤ 0,15 insgesamt, Rest Aluminium,
wobei das Walzprodukt einen porösen anodischen Oxidfilm aufweist, der elektrochemisch oder chemisch gefärbt ist, und wobei die Farbe der dekorativen Folie unterschiedlich ist, wenn sie in einem Einfallswinkel 0° und einem Einfallswinkel von 45° betrachtet wird, und **dadurch gekennzeichnet, dass** der poröse anodische Oxidfilm durch eine Sol-Gel-Beschichtung bedeckt ist, die vorzugsweise Silizium umfasst.

2. Produkt nach Anspruch 1, wobei Fe höchstens 0,5 Gew.-% beträgt und Si höchstens 0,3 Gew.-% beträgt.

3. Produkt nach Anspruch 1 oder Anspruch 2, wobei Mn höchstens 0,2 Gew.-%, Si höchstens 0,1 Gew.-% und Fe höchstens 0,2 Gew.-% beträgt.

4. Produkt nach Anspruch 1 oder Anspruch 2, wobei Mn: 0,8 - 1,5 Gew.-% und wobei der Mg-Gehalt höchstens 1,3 Gew.-% und vorzugsweise höchstens 0,6 Gew.-% beträgt.

5. Produkt nach einem der Ansprüche 1 bis 4, wobei der Si-Gehalt mindestens 0,03 Gew.-% beträgt.

6. Produkt nach einem der Ansprüche 1 bis 5, wobei der Fe-Gehalt mindestens 0,02 Gew.-% beträgt.

7. Produkt nach einem der Ansprüche 1 bis 6, wobei die Sperrschicht des porösen anodischen Oxidfilms eine Dicke von 15 bis 25 nm aufweist.

8. Produkt nach einem der Ansprüche 1 bis 7, wobei der poröse anodische Oxidfilm mindestens eines aus Zn, Ni, Sn, Co, Cu, Ag umfasst.

9. Produkt nach einem der Ansprüche 1 bis 7, wobei der poröse anodische Oxidfilm mindestens einen Farbstoff aus einem Azofarbstoff, einem Anthrachinonfarbstoff, und einem Indigofarbstoff umfasst.

10. Verfahren zur Herstellung eines eloxierten dekorativen Walzprodukts nach einem der Ansprüche 1 bis 9, die folgenden Schritte umfassend
- Gießen einer Aluminiumlegierung nach einem der Ansprüche 1 bis 6, zum Bilden eines Barrens;
- Wiedererwärmen und/oder Homogenisieren des Barrens vorzugsweise bei einer Temperatur von 460 °C bis 560 °C,
- Heißwalzen des Barrens auf eine endgültige Heißwalzdicke vorzugsweise bei einer Temperatur von 350 bis 500 °C,
- Kaltwalzen zum Erhalten eines kaltgewalzten Produkts mit einer bevorzugten endgültigen Dicke von 0,2 bis 2 mm und vorzugsweise von 0,5 bis 0,8 mm,
- optional Tempern des kaltgewalzten Produkts, vorzugsweise bei einer Temperatur von 200 bis 300 °C,
- Reinigen des kaltgewalzten Produkts, vorzugsweise mit einem Lösungsmittel oder einem wässrigen Reinigungsmittel, das Tenside enthält,
- optional Bereitstellen eines matten oder glänzenden Aussehens, beispielsweise durch Seidenmattätzen, oder durch chemisches/elektrochemisches Aufhellen,
- Eloxieren des kaltgewalzten Produkts in Schwefelsäure, Phosphorsäure, oder Oxalsäure oder einer Kombination daraus zum Erhalten eines porösen anodischen Oxidfilms,
- Färben des porösen anodischen Oxidfilms durch elektrochemisches Abscheiden, vorzugsweise von mindestens einem von Zn, Ni, Sn, Co, Cu, Ag von, oder chemischer Abscheidung von vorzugsweise mindestens einem Farbstoff aus einem Azofarbstoff, Anthrachinonfarbstoff, und Indigofarbstoff,
- Spülen mit entionisiertem Wasser,
- optional Versiegeln des porösen anodischen Oxidfilms durch hydrothermisches Versiegeln, Kaltversiegeln oder einer Kombination daraus,
- Trocknen,
- Beschichten des porösen anodischen Oxidfilms durch Abscheiden eines Sol-Gel-Vorläufers, gefolgt von Verdampfen und/oder Härten.

11. Verfahren nach Anspruch 10, wobei der Sol-Gel-Vorläufer aus einem Gemisch eines Polysiloxans gefertigt ist, vorzugsweise aus einer alkoholischen Lösung von Silan, bevorzugter aus einer alkoholischen Lösung eines Alkoxysilans und einer Wässrigen Lösung von kolloidalem Siliziumdioxid zubereitet ist.

12. Verfahren nach Anspruch 11, wobei der Sol-Gel-Vorläufer aus zwei Lösungen A und B zubereitet ist,
wobei Lösung A eine alkoholische Lösung aus einem oder mehreren Alkoxysilanen ist, der Alkohol, der als Lösungsmittel verwendet wird, Methanol, Ethanol, Propanol, vorzugsweise Isopropanol, Butanol oder eine Kombination daraus ist, die Alkoxysilane durch die allgemeine Formel XnSi(OR)4-n beschrieben sind, wobei "R" ein einfaches Alkyl ist, vorzugsweise ausgewählt aus der Gruppe bestehend aus Methyl, Ethyl, Propyl und Butyl und "X" auch ein Alkyl ist, vorzugsweise ausgewählt aus der Gruppe bestehend aus Methyl, Ethyl, Propyl und Butyl;
wobei Lösung B eine Lösung aus in Wasser gelöstem kolloidalem Siliziumdioxid ist.

13. Verfahren nach Anspruch 12, wobei die Alkoxysilane der Gruppe angehören, die Tetramethoxysilan (TMOS), Tetraethoxysilan (TEOS) und Methyltrimethoxysilan (MTMOS) umfasst.

14. Verfahren nach Anspruch 13, wobei die Lösung A 25 - 35 Gew.-% TEOS und 15 - 25 Gew.-% MTMOS umfasst, die beide in 40 - 60 Gew.-% Isopropylalkohol gelöst sind.

## Revendications

1. Produit laminé décoratif anodisé réalisé en un alliage d'aluminium constitué de, en % en poids,
Mg : de 0 à 1,5,
Mn : de 0 à 1,5,
avec Mg + Mn : de 0,5 à 3, et dans lequel
soit Mn : de 0,8 à 1,5
soit Mg : de 0,5 à 1,1 et Mn ≤ 0,2,
Si : ≤ 0,6,
Fe : 0,8,
Ti : ≤ 0,1,
Cu : ≤ 0,3,
Cr: 0,1,
Zn : ≤ 0,25,
Zr : ≤ 0,1,
d'autres éléments ≤ 0,05 chacun et ≤ 0,15 au total, le reste étant de l'aluminium, dans lequel le produit laminé possède un film d'oxyde anodique poreux qui est coloré de manière électrochimique ou chimique et dans lequel la couleur de la feuille décorative est différente si elle est vue selon un angle d'incidence de 0° et selon un angle d'incidence de 45° et
**caractérisé en ce que** le film d'oxyde anodique poreux est recouvert par un revêtement sol-gel comprenant de préférence du silicium.

2. Produit selon la revendication 1 dans lequel Fe représente au plus 0,5 % en poids et Si représente au plus 0,3 % en poids.

3. Produit selon la revendication 1 ou la revendication 2 dans lequel Mn représente au plus 0,2 % en poids, Si représente au plus 0,1 % en poids et Fe représente au plus 0,2 % en poids.

4. Produit selon la revendication 1 ou la revendication 2 dans lequel Mn : de 0,8 à 1,5 % en poids et dans lequel la teneur en Mg représente au plus 1,3 % en poids et de préférence au plus 0,6 % en poids.

5. Produit selon l'une quelconque des revendications 1 à 4 dans lequel la teneur en Si représente au moins 0,03 % en poids.

6. Produit selon l'une quelconque des revendications 1 à 5 dans lequel la teneur en Fe représente au moins 0,02 % en poids.

7. Produit selon l'une quelconque des revendications 1 à 6 dans lequel la couche barrière du film d'oxyde anodique poreux possède une épaisseur de 15 à 25 nm.

8. Produit selon l'une quelconque des revendications 1 à 7 dans lequel le film d'oxyde anodique poreux comprend au moins l'un parmi Zn, Ni, Sn, Co, Cu, Ag.

9. Produit selon l'une quelconque des revendications 1 à 7 dans lequel le film d'oxyde anodique poreux comprend au moins un colorant parmi un colorant azoïque, un colorant anthraquinone, un colorant indigo.

10. Procédé pour réaliser un produit laminé décoratif anodisé selon l'une quelconque des revendications 1 à 9 comprenant les étapes de
- coulée d'un alliage d'aluminium selon l'une quelconque des revendications 1 à 6 pour former un lingot ;
- réchauffage et/ou homogénéisation du lingot de préférence à une température de 460 °C à 560 °C,
- laminage à chaud du lingot jusqu'à une épaisseur finale de laminage à chaud de préférence à une température de 350 à 500 °C,
- laminage à froid pour obtenir un produit laminé à froid, ayant une épaisseur finale préférée de 0,2 à 2 mm et de préférence de 0,5 à 0,8 mm,
- facultativement, recuit dudit produit laminé à froid de préférence à une température de 200 à 300 °C,
- nettoyage dudit produit laminé à froid, de préférence avec un solvant ou un nettoyant aqueux contenant des tensioactifs,
- facultativement, fourniture d'un aspect mat ou brillant par exemple par gravure satinée mate ou par brillantage chimique/électrochimique,
- anodisation dudit produit laminé à froid dans de l'acide sulfurique, de l'acide phosphorique ou de l'acide oxalique ou une combinaison de ceux-ci pour obtenir un film d'oxyde anodique poreux,
- coloration dudit film d'oxyde anodique poreux par dépôt électrochimique de préférence d'au moins l'un parmi Zn, Ni, Sn, Co, Cu, Ag ou dépôt chimique de préférence d'au moins un colorant parmi un colorant azoïque, un colorant anthraquinone, un colorant indigo,
- rinçage avec de l'eau désionisée,
- facultativement, colmatage du film poreux d'oxyde anodique par colmatage hydrothermal, colmatage à froid ou une combinaison de ceux-ci,
- séchage,
- revêtement du film poreux d'oxyde anodique par dépôt d'un précurseur de sol-gel suivi par une évaporation et/ou un durcissement.

11. Procédé selon la revendication 10 dans lequel le précurseur de sol-gel est réalisé à partir d'un mélange d'un polysiloxane, de préférence préparé à partir d'une solution alcoolique d'un silane, plus préférablement à partir d'une solution alcoolique d'un alcoxysilane, et d'une solution aqueuse de silice colloïdale.

12. Procédé selon la revendication 11 dans lequel le précurseur de sol-gel est préparé à partir de deux solutions A et B,
la solution A étant une solution alcoolique d'un ou de plusieurs alcoxysilanes, l'alcool utilisé comme solvant étant le méthanol, l'éthanol, le propanol, de préférence l'isopropanol, le butanol ou une combinaison de ceux-ci, les alcoxysilanes étant décrits par la formule générale XnSi(OR)4-n où « R » est un alkyle simple, de préférence choisi parmi le groupe constitué du méthyle, de l'éthyle, du propyle et du butyle et « X » est également un alkyle, de préférence sélectionné parmi le groupe constitué du méthyle, de l'éthyle, du propyle et du butyle ;
la solution B étant une solution de silice colloïdale dissoute dans l'eau.

13. Procédé selon la revendication 12, dans lequel lesdits alcoxysilanes appartiennent au groupe comprenant le tétraméthoxysilane (TMOS), le tétraéthoxysilane (TEOS) et le méthyltriméthoxysilane (MTMOS).

14. Procédé selon la revendication 13, dans lequel la solution A contient de 25 à 35 % en poids de TEOS et de 15 à 25 % en poids de MTMOS, tous les deux dissous dans 40 à 60 % en poids d'alcool isopropylique.
